

June 4, 1940.

E. WEISS

2,203,375

PROCESS FOR MERCERIZING FABRIC

Filed May 24, 1939



INVENTOR

ERNST WEISS.

BY

Ward, Crosby & Neal

ATTORNEYS

## UNITED STATES PATENT OFFICE

2,203,375

## PROCESS FOR MERCERIZING FABRIC

Ernst Weiss, Bunt, Wattwil, Switzerland, assignor  
to Heberlein Patent Corporation, New York,  
N. Y., a corporation of New York

Application May 24, 1939, Serial No. 275,478  
In Germany October 15, 1937

4 Claims. (Cl. 8—125)

This invention relates to process for mercerizing fabrics.

More particularly the invention relates to the production of improved fabrics—piece goods—containing vegetable fibers and having the following characteristics, i. e., a good quality of sheen or lustre; the finished fabric having, at least in one direction, that is either along the warp or weft, an increased dimension as compared with the corresponding dimension of the original fabric before treatment, the character of the mercerized fabric being such that even with the increased dimension the fabric has substantially improved stability against shrinkage. Preferably such dimension is increased sufficiently and the finished fabric is of such character that even if, subsequent to the mercerizing process, the fabric is subjected to several washing tests or to mechanical shrinkproofing treatments such as the Sanforizing treatment, it will still maintain an increased dimension in the stretched direction greater than the original dimension of the fabric before treatment, while maintaining the other good qualities of mercerized fabric such for example as tensile strength. It is a particularly valuable characteristic of the invention that notwithstanding such increased dimension, the fabrics treated according to this process are effectively stabilized in their dimensions and therefore shrink only to a comparatively slight or negligible degree upon being subsequently subjected to repeated washing. Such fabric when produced according to the preferred manner of carrying out the process, has in addition to the above set forth characteristics, a strikingly high mercerization sheen and softness.

With preferred practices of the process, one dimension, for example, the warp, may be substantially increased, while the weft dimension may be retained at least as large as is possible with former mercerization processes; and such reduction as occurs in the weft dimension may in general be compensated for or substantially offset by the enlarged warp dimension. This is of substantial commercial importance in that with the usual mercerization processes as heretofore practiced, the area of the finished fabric, after the mercerization, is substantially less than that of the original untreated material, and furthermore, when the usual mercerized fabric is washed or subjected to a shrinkproofing treatment, its area is even further substantially reduced. These facts greatly increase the real cost of the usual mercerization treatment. Thus, the costly loss in area of the material, as well as its

shrinkable character after the usual mercerization treatment, tend to diminish to a substantial extent the advantages of mercerization. On the other hand, with fabrics made according to the preferred practice of the present invention, these disadvantages of mercerization are not only eliminated, but the permanent gain in yardage, as a practical matter, may be sufficient in value to offset, at least to a considerable extent, the cost of the treatment; at the same time greatly improving the product as compared with mercerized fabrics heretofore available.

Generally stated, these results are made possible by conducting the mercerizing treatment in such manner that the fibers are first quickly, thoroughly and effectively impregnated substantially throughout with a caustic solution of mercerization strength, before the fibers are substantially swelled by the caustic, then while subjecting to caustic, permitting the fiber to thoroughly swell, substantially completely and homogeneously, and then tensing the fabric while it is in this state of maximum swelling; the tension being applied in such manner that it is greatest in the direction of the yarn which is mainly to impart sheen, and in this direction being of such force as to stretch the fabric beyond its original dimension (before shrinkage), and according to the preferred process, to a point beyond the elastic limit of the swelled fibers and between this limit and the breaking or tearing limit of the fabric, and retaining (but not increasing) substantially the full dimensions of the fabric produced by such tensing, while the fabric is thereafter being freed of the caustic solution and preferably also during teneting and finishing.

The invention consists in the novel process or combinations of process steps hereinafter more fully described by way of examples according to the preferred manner of execution, and will be more particularly pointed out in the appended claims.

The drawing schematically illustrates one form of apparatus by way of example, which may be used for carrying out the process of the invention.

The original material to be treated according to this invention may be a fabric comprising or containing vegetable fibers, such as fabrics made of cotton, hemp, flax, linen, jute, or ramie, as well as mixed fabrics made of these materials, or these materials mixed with animal fibers such for example as silk, artificial silk, or spun rayon made of regenerated cellulose or cellulose derivatives.

The material to be treated, preferably while

in the dry state, is first subjected to a penetrating impregnation with a caustic solution of mercerizing strength, such penetration being forcefully effected, preferably mechanically, with sufficient rapidity and thoroughness so as to enable subsequent substantially complete homogeneous swelling of the fiber. Such penetration should be effected while the fabric is not under substantial tension, more particularly at least longitudinally of the yarn which is to mainly impart the mercerization sheen. After such impregnation, the fiber of the fabric is permitted to homogeneously swell to substantially the maximum extent possible from such impregnation and subsequent application of the caustic and is allowed to shrink during the swelling, and when the fiber has reached such condition of maximum swelling, the fabric is overstretched by the application of tension, preferably beyond the elastic limits of the fiber and greatly in excess thereof, and preponderantly in the direction of the yarn which is to mainly impart the sheen; the overstretches usually being from 3 or 4 to 7%. Thereupon while the dimensions of the fabric resulting from such overstretches are substantially maintained, the fabric is freed from the caustic solution tentered and finished in the usual manner.

In performing the process, it is particularly important that the fiber of the fabric be thoroughly, completely and homogeneously swelled, that is, thoroughly mercerized. To this end it is important that the impregnation precede any substantial swelling. Otherwise, if the swelling begins in the outer layers of the yarn to any substantial degree before the complete impregnation, a deeper impregnation will thereby be checked or made impossible, due to the fact that the yarns are made less permeable to the caustic. Accordingly the impregnation should be effected extremely rapidly and uniformly, since this will subsequently permit a completely homogeneous swelling, difficult or impossible to otherwise achieve. The forcefully effected impregnation may therefore preferably be aided before the commencement of the swelling by the addition to the caustic solution of suitable wetting agents or mercerization adjuvants such as a material known in the trade as "mercerol" (a mixture of crude cresol with fat solvents such for instance as "cyclohexanol"); but the wetting agents alone are not sufficient to give the necessary quick and thorough penetration, it being necessary to use for this purpose an effective forceful impregnation preferably by mechanical means such for example as by a pair of squeezing rollers between which the fabric is pressed through in the presence of the mercerizing agent. The impregnation process may also be promoted by subjecting the goods to a vacuum followed by wetting the fabric with a mercerizing caustic solution under pressure.

With prior mercerization practices it is customary to speak of the "degree of mercerization," thereby recognizing that with the usual practice of mercerizing, a completely homogeneous thorough swelling is not necessary. With the process of the present invention, however, a substantially complete and homogeneous thorough swelling appears to be very important, since otherwise the necessary degree of plasticity of the fiber is not obtained for rendering it possible to properly stabilize the dimensions of the strongly overstretched fabric, in accordance with the invention.

As above stated, the material is permitted to shrink during the swelling stage of the process. While in prior known mercerization processes such a shrinking step in the procedure is left optional and is therefore not required, this mode of operation has been found to be important with the present invention in order to obtain the desired effects in the finished fabric. 5

The specific composition of the caustic solution may be determined according to the particular properties of the goods being treated and in accordance with the known procedure for mercerizing the same. 10

In practicing the present invention, it is important that the over-stretching of the fabric 15 take place at a time when the fiber is swelled to substantially the maximum amount, as distinguished for example from prior processes in which the stretching may be done during reduction of the swelling, and as for instance during 20 the removal of the caustic solution. While in the known mercerizing processes the stretching may take place before, during or after the mercerizing, that is, prior to the removal of the 25 caustic solution or else during the removal thereof, the stretching during the removal of the caustic solution is frequently preferred because less power is required therefor at this stage. In short, for the mercerizing effects heretofore achieved, 30 it made little difference whether the tensioning of the fabric took place before or during the removal of the caustic solution. On the other hand, with the present invention, it has been found to be impossible to attain the desired and effective 35 stabilization of the fabric against shrinkage if the tensioning is not effected during the time that the fabric is in substantially its maximum swelled condition. That is, the tensioning should be applied at a time when the complete fiber 40 has a high degree of plasticity and not before this stage or after such plasticity has been disturbed by the reduction of the swelling. If the stretching should take place while the caustic is 45 being washed out, then the fabric will shrink badly in subsequent washings of the finished fabric.

Both the preliminary shrinking and the tensioning of the fabric are effected preponderantly in a direction lengthwise of the yarn which is mainly to impart the sheen. That is, the direction is determined by the nature of the fabric, or whether the yarn which is to impart the sheen is located in the warp or in the weft (for example warp satin or weft satin). In the case of muslin, where the warp and weft yarns are almost equivalent, and linen binding is present, the direction of the shrinking and overstretches is optional. 50

As above indicated, in accordance with the invention the fabric is stretched at least in one direction, or preponderantly in one direction, beyond the corresponding original dimension of the fabric, i. e., "overstretched". In older publications on mercerization, it is mentioned, to be sure, that it is possible to stretch beyond the 65 original dimension, but there only a few percent at most could have been involved since at that time it was difficult with the machines available or which could then be built, to stretch the fabric even to the original length. And the treatments were not such that the gain could be maintained or stabilized. A more recent disclosure describes a process for the mercerization of cotton, wherein yarn is permitted to shrink and is subsequently temporarily stretched to about 4% 70

75

5 beyond its original length. In this case, also, no stabilization of the yarn length is effected, since the caustic is washed out during the stretching, and the stretched dimensions are not maintainable for various reasons, and the completed product is specified as having its original dimensions.

10 According to the preferred practice of the present invention the stretching is effected by applying to the fabric, tension sufficient to exceed the "flow limits" or elastic limit of the swelled fibers, but below the breaking limits thereof. The "flow limits" or elasticity limits may be defined as the limits reached when the tension applied causes the elastic deformation 15 (reversible elongation) of the fibers to pass over into permanent deformation (irreversible elongation); that is, limits at which the deformation no longer substantially disappears after discontinuance of all imposed tensions. The breaking 20 limits may be defined as the limits at which the tensions applied are such as to cause tearing of the fabric or substantial damage to the fibers thereof.

25 As above indicated, while the material is being freed from the caustic solution, tentered and finished, its increased dimensions as fixed during its state of maximum swelling or plasticity, are to be retained as nearly as possible. It is particularly important to retain the enlarged dimensions 30 during removal of the caustic solution. This condition may preferably be fulfilled by using for the tensioning, chain mercerizing equipment in which the fabric dimensions remain constant without further trouble. One may for example use a well-known form of chain-mercerizing machine upon replacing the customary foulard equipment with a suitable impregnating assembly and by performing the various process steps so as to carry out the invention as above 35 described. In order to obviate tearing of the goods at the pincers during the strong over-stretching, the fabric may for example be conveyed to the pincer chains in a previously tensed state, by stretching it for example by means of 40 two pairs of squeezing rollers having respectively 45 different speeds, i. e., the second pair having a more rapid drive.

50 The requirement of retaining the dimensions during the removal of the caustic solution may be also fulfilled by using chainless mercerizing machines, if for example, the spreading rollers of the apparatus for removal of the caustic solution may be individually driven in such way that during a given interval of time substantially 55 identical fabric areas will run over all of the rollers. The rollers of course should be arranged in such a way that slipping of the fabric thereon is precluded. Accordingly, in case the rollers are all of the same dimensions, for example, they 60 should be driven at equal speeds.

60 Fabrics which have been ennobled or finished according to the preferred execution of this invention, are distinguishable by the strikingly high sheen or light reflection given in the direction of and by the over-stretched yarns of the fabric, and by the soft pleasant feel of the fabric, whereas certain of their other important textile properties, as for instance their tensile strength, remain the same or as good as before the treatment. One of the most conspicuous features of 65 the product, however, is its comparative freedom from shrinking despite the very substantial over-stretching of the fabrics treated in accordance with the invention. That is, the finished fabric 70 will shrink but slightly on being repeatedly

washed, even along the direction of the predominant overstretching. Thus in this direction at least, there persists even after washing, an increased dimension which may be regarded as a gain in the fabric yardage available from the use 75 of the process. This gain becomes particularly apparent when the process in accordance with the invention is combined with an immediately succeeding shrinkproofing process such for example as well-known mechanical shrinkproofing 10 processes (such as Sanforizing). Whereas, when such mechanical processes have heretofore been applied to fabrics containing vegetable fiber a substantial loss of yardage, as a result of shrinking 15 of the goods, has had to be accepted as a foregone conclusion, yet when such a mechanical process is applied to the overstretched fabrics as a part of the present invention, not only is such loss due to shrinkage avoided, but an actual 20 increase or gain in the yardage of the final fabric may be accomplished.

Further treatments and completion of the fabric which has been treated in accordance with the invention may be effected in desired well-known ways. In particular the bleaching and 25 bucking of the material may be effected at any desired stage, i. e., before or after the mercerization treatment according to the invention.

The drawing schematically illustrates one suitable form of apparatus by way of example only, 30 with which the process may be carried out with a chainless mercerizing type of machine, but the invention is not to be limited by or to such machine. The fabric 10 may pass over suitable guide or idler rollers 11 into a vat 12 containing 35 the mercerizing solution including the wetting agents or mercerization adjuvants. As shown the fabric in passing over a roller 13 becomes immersed in the solution and wetted, the fabric being preferably dry when it enters the solution. 40 Having the fabric substantially dry when it enters the bath is desirable in producing the fullness and soft hand of the fabric. Almost immediately thereafter it is fed through a pair of squeezing rollers as at 14 for promoting intensive 45 mechanical impregnation before the swelling action has opportunity to take place and while being free of any substantial tension. After leaving the squeezing rollers 14, the fabric may pass over an assembly of rollers 15 within the 50 vat 12, and it is upon these rollers that the homogeneous swelling of the fiber takes place. In passing from the rollers 14 to the rollers 16 the fabric is allowed to shrink. In case the shrinkage is desired preponderantly in the warp direction, which is advantageous, then the rollers 14 will be driven with a surface speed slightly faster 55 than those of the subsequent rollers in the vat 12, and so that the fabric is advanced without any substantial lengthwise tension. 60

Upon leaving the vat 12, the fabric is suitably guided to and between a pair of driven squeezing rollers 16, at which time the condition of maximum swelling has been reached. From the squeezing rollers 16, the fabric is subjected to a 65 powerful lengthwise tension as it passes over guide roller 17, and spreader rollers 18. On the way from the rollers 15 to the squeezing rollers 16 and thence over the guide roller 17, the fabric, in this particular machine, has opportunity to 70 shrink in the direction of the weft. As the material passes over the spreader rollers 18, it is also subjected to transverse tensioning as well as the lengthwise tensioning. The speed of the fabric is such in any case as to allow the caustic to 75

act for a sufficient time to bring about the desired thorough swelling. As the fabric leaves the rollers 18, it has the desired overstretched dimensions, preferably mainly along the warp, and such dimensions are retained during passage of the material over an assembly of rollers 19. By regulating the surface speed of the rollers 19 as compared with that of the rollers 16, the direction of the predominant stretch (along the warp or the weft) and the degree of stretching may be regulated to some extent. Further regulation is possible by varying the character and numbers of the rollers 18, or by varying the winding angle of the fabric in respect to the rollers 16 (i. e., the position of each of rollers 18 in respect to the next, may be varied).

While passing over the rollers 19, the caustic solution may be removed from the fabric in any desired well-known way as for example by spraying with hot water from spray pipes 20. To insure that the finished fabric will be of a soft character with a high sheen, it is important to effect the washing at a temperature of at least 80° C.

35 The spreader rollers 18 may be so formed as to transversely tension the fabric to the desired extent while permitting of the desired lengthwise tensioning caused by the rollers 16 and 19. The rollers 19 may be of such dimensions, shape and form as to maintain constant, the lengthwise and transverse dimensions of the fabric, substantially the same as when it leaves the rollers 18. The rollers 19 are accordingly preferably all alike and driven at the same speed.

During the lixiviation at rollers 19, the tensions in the fabric decrease, and after the lixiviation only a small pull is necessary to retain the fabric dimensions. The same is true during any subsequent finishing operations. As stated, the tension of the fabric during the washing must be such that there is no stretching of the fabric. The fabric will finally leave the apparatus by passing between a pair of rollers as at 24, so driven as to cooperate with the rollers 19 in maintaining constant the dimensions of the fabric after lixiviation. The more perfectly its dimensions are kept constant during removal of the caustic solution, the less the completed fabric will shrink upon being washed. As stated, these 50 dimensions are also preferably maintained during subsequent tentering and finishing.

Obviously the practice of the process in accordance with the invention is not limited to the use of the particular form of apparatus here described and shown.

The following are specific examples of the process of the invention as we now prefer to carry it out. It is to be understood that the invention is not limited to any of the particular examples hereinafter given, except as indicated in the appended claims:

Example 1.—A poplin fabric may be thoroughly and homogeneously mercerized for example, by using apparatus such as shown in the drawing, and with a caustic solution comprising sodium hydroxide of 30° Bé. at a temperature of 15-20° C., to which is added a wetting agent or a mercerization adjuvant amounting, for example, to 2% of the solution, if mercerol is used. 65 The solution is allowed to act for from 15 to 25 seconds between rollers 13 and 16, which is the time required in this example for complete swelling prior to stretching, but the time may be somewhat longer if desired. Suitable periods of 70 time for the travel of the fabric between other

parts of the apparatus shown will then occur if the distances between the various rollers are proportioned substantially according to the drawing. The material is so conducted through the apparatus that the fabric may first shrink quite freely (i. e., up to rollers 16), preponderantly in the warp direction for example. This is followed by a powerful stretching at a time when the fabric has reached the condition of maximum swelling (for example between rollers 16 and 19) and with tension sufficient to increase the length of the fabric by about 7% or more, up to nearly 10%. For attaining the highest sheen with stabilized overstressing the tension should be sufficient to increase the length by about 7% or over; for the attainment of stabilized overstressing with somewhat less sheen the fabric may be overstressed to a less extent.

With a typical poplin fabric of 85 cm. width, a longitudinal pull of 180 kilograms caused an elongation of 7% when the fabric was in maximum swollen condition. The force required will of course very considerably, depending upon the characteristics of each particular fabric, but preferably should greatly exceed that required to stretch the fabric to its elastic limit. Usually, however, an elongation of 9% cannot be exceeded without danger of tearing or injury to the fabric. During the longitudinal stretching a powerful tension is also applied transversely of the 3 fabric (as by spreader rollers 18). The time during which the fabric travels from the point where the longitudinal stretching force is first applied (as at rollers 16) to the point where transverse stretching of the fabric is completed (as at the 36 last of rollers 18), may be from 10 to 15 seconds. Immediately thereafter the fabric is freed from the caustic solution, as by lixiviation with water at or above 80° C., then tendered and finished, while maintaining as nearly as possible the 40 same dimensions of the fabric as resulted from the powerful stretching.

Fabrics which have been treated in accordance with this example have an increased length of from about 7 to nearly 10% as compared with 45 the untreated goods. At the same time the width of the fabric may be maintained as free of shrinkage as with mercerization processes heretofore known, i. e., the loss in the width need not exceed about 4 to 5%. Hence, in some cases the 50 total area of the fabric may even be enlarged. In typical cases the area is from 1 to 3% greater than obtainable with the normal mercerization treatments of the same fabric. Also the resulting product will have a high mercerization sheen, 55 beyond that heretofore attained, as well as having a noticeably softer feel. The improved sheen is immediately noticeable to the eye, in comparison with the same product treated according to mercerization processes as heretofore used.

Measurements of lustre according to Sommers' method have been made of this improved product in comparison with the same material which had been treated in accordance with prior known practices to give what has heretofore been considered a beautiful mercerization sheen. These 65 tests reveal that with the incident light beam directed along the strongly overstretched yarns, the maximum degree of lustre resulting with this example of the invention is about three times higher than obtainable with the prior mercerization procedure. Also with the incident light directed along the yarns which had not been so strongly tensioned, the degree of lustre was superior in the case of the product made according to this 70 75

- invention. The tests also reveal that with the product of the invention, the degree of lustre varies much more sharply, depending upon the angle of incidence of the light, which fact is also clearly noticeable to the eye in comparing the finished fabrics and serves to give the fabrics treated according to the invention, striking variations in brightness upon changes in the position thereof in respect to the incident light.
- 10 Microscopic examination of the cross section of the fibers of fabric treated in accordance with the preferred execution of the above described process, reveals that the cross sections of a large portion of the individual fibers have somewhat polyhedral outlines as compared with more smoothly curved outlines of fibers as ordinarily mercerized. Furthermore, with the improved process, the degree of swelling of the various fibers as well as within each fiber is appreciably more uniform.
- 15 20 The cross sections although polyhedral are more swelled out toward a circular form as contrasted with the case of ordinary mercerization where the shapes of the cross sections are preponderantly elliptical or kidney shaped, less uniform, and smaller. With the usual mercerization procedure, many of the fibers have a somewhat ribbon-like appearance, but with the improved process there are very few fibers with such ribbon-like structure.
- 25 30 Although with the usual mercerization processes, the degree of mercerization is sometimes estimated by determining the ratio of the amount of dyestuff, such as benzopurpurine 4B, which will be taken up by the untreated fabric as compared with the same fabric mercerized (more dyestuff being absorbed the greater the degree of mercerization), it has been found that fabrics treated in accordance with the preferred execution of the present invention absorb less of such dyestuff than normally mercerized fabrics, notwithstanding the greatly improved mercerization sheen.
- 35 40 In spite of the fact that the fabric has been strongly overstretched, standard washing tests reveal that it does not shrink in length more than about 2 to 3% as compared to its length prior to the washing. If the fabric as mercerized is subjected to a mechanical shrinking process, for instance such as Sanforizing, the Sanforized fabric may still show an increase in length of about 5 to 7% as compared with the original untreated goods. After washing the Sanforized product six times, the shrinkage tolerance of 1% is not exceeded. The Sanforizing process referred to is a well-known one and may be such as disclosed in the following patents, reference to which is hereby made: United States Patents Nos. 1,861,423, 1,861,424, 2,037,676 and 2,082,981.
- 45 50 55 With the mercerization processes heretofore used, the length of the fabric is not increased beyond 3% and generally only 1%, and when such a fabric has been subjected to washing tests or Sanforizing, it will usually show a loss of from 3 to 6%; which means that the fabric will show a loss, from its original length in the gray, of from 2 to 3%, or often even as much as 5%.
- 60 65 70 75 Example 2.—A muslin fabric may be treated, for example, by using apparatus such as shown in the drawing, and generally in accordance with the process of Example 1, except that the longitudinal stretching may be such as to effect an elongation of 4 to 6% and with a transverse spreading of the fabric somewhat greater than Example 1. These differences from Example 1 are advisable because in the case of muslin, the
- yarn which imparts the sheen is ordinarily distributed about equally in the warp and the weft. The fabric shows an increased silk-like lustre and the yarns seem to be thinner and the fabric somewhat finer in comparison with ordinary mercerization.
- 75 80 85 90 95 Example 3.—A "limberic" fabric may be treated in accordance with the same principles stated above in connection with the muslin fabric of Example 1. Here the yarns which predominantly impart the sheen are run in the direction of the filling and accordingly in the mercerization bath, the fabric should be allowed to shrink predominantly along the direction of the weft, and the over-stretching should be also predominantly along the direction of the weft. The fabric shows an increased silk-like lustre and the feel is characterized by an increased softness and pliability in comparison with ordinary mercerization. The above mentioned stabilized character of the fabric to resist substantial shrinkage is also present in the fabric made according to this example, so that even after washings or Sanforizing a gain in the stretched dimension is maintained over that in the original fabric prior to mercerization.
- 95 100 105 110 115 This invention does not reside merely in stretching the fabric during mercerization beyond the original dimension, but it resides, as to the product, in the peculiar, new and valuable character of the finished mercerized fabric which gives it a good sheen (and in the preferred form of the invention a very high sheen and softness) and enables it to resist shrinkage to such an extent that after repeated washing tests or after Sanforizing, it loses only about 2 to 3% of its length, and this is true even in cases where in the mercerization treatment the fabric had been stretched to a finished length of several percent beyond its original or gray length.
- 115 120 125 130 135 While the invention has been described in detail with respect to particular preferred examples, it will be understood by those skilled in the art after understanding the invention that various changes and further modifications may be made without departing from the spirit and scope of the invention, and it is intended therefore in the appended claims to cover all such changes and modifications.
- 135 140 145 150 155 This application is a continuation in part of my copending application Serial No. 217,646, filed July 6, 1938.
- 155 160 165 170 175 What is claimed as new and desired to be secured by Letters Patent is:
1. Process of finishing a fabric containing vegetable fiber to obtain a good mercerization sheen and improved stability against shrinkage by subsequent washings, which comprises quickly effecting a thoroughly penetrating impregnation of the fiber with a caustic mercerization solution, such thorough penetration being effected before substantial swelling of the fiber takes place so as to enable subsequent thorough and homogeneous swelling, then continuing the action of the caustic under conditions permitting the fiber to substantially homogeneously and thoroughly swell to substantially the maximum extent the fibers during the swelling being allowed to shrink mainly in a direction of the yarn which is to principally impart the sheen, then "overstretching" the fabric while in such substantially maximum swelled condition to a point beyond the corresponding original dimension of the fabric but not exceeding 8% beyond said original dimension, by tensioning the fabric preponderantly in said direction, and thereafter removing the caustic

solution from the fabric while maintaining substantially its dimensions resulting from said overstretching.

2. Process of finishing a fabric containing vegetable fiber to obtain a good mercerization sheen and improved stability against shrinkage by subsequent washings, which comprises quickly effecting a thoroughly penetrating impregnation of the fiber with a caustic mercerization solution, such 5 thorough penetration being effected before substantial swelling of the fiber takes place so as to enable subsequent thorough and homogeneous swelling, then continuing the action of the caustic under conditions permitting the fiber to substantially 10 homogeneously and thoroughly swell to substantially the maximum extent, the fibers during the swelling being allowed to shrink mainly in a direction of the yarn which is to principally 15 impart the sheen, then "overstretching" the fabric while in such substantially maximum swelled condition and to a gain of about 3 to 8% in such direction, by tensioning the fabric preponderantly in said direction, and thereafter removing the caustic solution from the fabric while 20 maintaining substantially its dimensions resulting from said overstretching.

3. Process of finishing a fabric containing vegetable fiber to obtain a good mercerization sheen and improved stability against shrinkage by subsequent 25 washings, which comprises quickly effecting a thoroughly penetrating impregnation of the fiber with a caustic mercerization solution, such thorough penetration being effected before substantial swelling of the fiber takes place so as to enable subsequent thorough and homogeneous swelling, then continuing the action of the caustic under conditions permitting the fiber to substantially 30 homogeneously and thoroughly swell to substantially the maximum extent, the fibers during the swelling being allowed to shrink mainly 35 in a direction of the yarn which is to principally impart the sheen, then "overstretching" the fabric while in such substantially maximum swelled condition and to a gain of about 5 to 8% by tensioning the fabric preponderantly in said direction, and by applying sufficient tension transversely of said direction to prevent transverse shrinkage in excess of about 5%, and thereafter removing the caustic solution from the fabric while maintaining substantially its dimensions resulting from said overstretching.

substantially the maximum extent, the fibers during the swelling being allowed to shrink mainly in a direction of the yarn which is to principally impart the sheen, then "overstretching" the fabric while in such substantially maximum swelled condition and to a gain of about 3 to 8% in such direction, by tensioning the fabric preponderantly in said direction, and thereafter removing the caustic solution from the fabric by hot lixiviation while maintaining substantially 10 its dimensions resulting from said overstretching.

4. Process of finishing a fabric containing vegetable fiber to obtain a good mercerization sheen and improved stability against shrinkage by subsequent washings, which comprises quickly effecting a thoroughly penetrating impregnation of the fiber with a caustic mercerization solution, such thorough penetration being effected before substantial swelling of the fiber takes place so as to enable subsequent thorough and homogeneous 20 swelling, then continuing the action of the caustic under conditions permitting the fiber to substantially homogeneously and thoroughly swell to substantially the maximum extent, the fibers during the swelling being allowed to shrink mainly 25 in a direction of the yarn which is to principally impart the sheen, then "overstretching" the fabric while in such substantially maximum swelled condition and to a gain of about 5 to 8% by tensioning the fabric preponderantly in said 30 direction, and by applying sufficient tension transversely of said direction to prevent transverse shrinkage in excess of about 5%, and thereafter removing the caustic solution from the fabric while maintaining substantially its dimensions resulting from said overstretching.

ERNST WEISS.

CERTIFICATE OF CORRECTION.

Patent No. 2,203,375.

June 4, 1940.

ERNST WEISS.

It is hereby certified that error appears in the printed specification of the above numbered patent requiring correction as follows: Page 3, first column, line 4, for "strteched" read --stretched--; line 72, for "shrink-  
ling" read --shrinking--; page 4, first column, line 13, for "numbers" read  
--number--; and second column, line 39, for "tendered" read --tentered--;  
page 5, second column, line 66, claim 1, after "extent" insert a comma;  
and that the said Letters Patent should be read with this correction there-  
in that the same may conform to the record of the case in the Patent Office.

Signed and sealed this 6th day of August, A. D. 1940.

Henry Van Arsdale,

Acting Commissioner of Patents.

(Seal)